

April 4, 1939.

W. H. BURKHART ET AL

2,152,788

SOAP PRODUCT AND THE MANUFACTURE THEREOF

Original Filed May 24, 1933

2 Sheets-Sheet 1

Fig.1.



Fig.2.



INVENTORS  
William H. Burkhardt and  
Eugene T. Marceau  
BY  
E. C. Sanborn  
ATTORNEY

April 4, 1939.

W. H. BURKHART ET AL

2,152,788

SOAP PRODUCT AND THE MANUFACTURE THEREOF

Original Filed May 24, 1933

2 Sheets-Sheet 2

Fig. 5



Fig. 3



Fig. 4



Inventor

William H. Burkhart  
and  
Eugene J. Marceau  
E. C. Sanborn

Attorney

## UNITED STATES PATENT OFFICE

2,152,788

SOAP PRODUCT AND THE MANUFACTURE  
THEREOF

William H. Burkhart, Baltimore, Md., and  
Eugene T. Marceau, Maplewood, N. J., assign-  
ors to Hecker Products Corporation, a corpo-  
ration of New Jersey

Application May 24, 1933, Serial No. 672,724  
Renewed September 23, 1938

15 Claims. (Cl. 87—16)

This invention relates to a novel spray dried soap product and the manufacture thereof. Various prior spray dried soap products in flake or particle form have been found objectionable as not soluble with sufficient rapidity and completeness, as of undesirable bulking weight, or as containing excessive proportions of dust. Attempts to overcome these objections have resulted in the production of particles of rounded or generally globular character and containing definite interior voids surrounded by walls or shells of solidified soap material. In the preparation of such products soap compositions are sprayed into air currents which are at such high temperatures adjacent the spray nozzles as to generate steam within the particles with consequent pronounced inflation thereof. The resultant rounded void-containing shell-like particles, while possessing the advantage of low bulking weight, involve certain disadvantages. For example, they exhibit surfaces of vitrified character which impede their solubility. Also, due to the necessity of expanding such particles to obtain low bulking weight by means of generating steam internally within them, excessively high temperatures (in the neighborhood of 400° F. or higher) are employed, but only a small amount of the available heat is usefully absorbed in the process and the major part is wasted.

Again, the processes commonly employed for the production of the rounded shell-like steam-expanded particles of the prior art involve the injection of the soap paste into the stream of heated air or gas at its hottest point in the spray tower, whereupon the moisture in the injected particles is vaporized with resultant violent inflation of the particle and escape of almost all of its moisture. The bead-like puffed particles resulting are undesirably low in moisture content.

Such processes, moreover, as a result of their employment of heated air both as a drying medium and as a means for puffing the particles by steam generation, do not lend themselves readily to variations in the rate of production and at the same time to control of the bulking weight and moisture content of the product.

The present invention follows from our discovery that particles of rounded or globular void-containing formation are not necessary to the attainment of a satisfactory and efficient soap product overcoming the deficiencies of previous soap compositions. This invention provides a product comprising agglomerations of particles aggregated together to form networks of sponge or coral-like character in marked contrast to

the hollow bead or shell-like soap products with interior voids which have heretofore been deemed essential for a satisfactory flaked or powder-like soap material. In the novel product forming the subject of this invention, desirable low bulking weight is obtained without the generation of steam within the particles. Due to its aggregated sponge or coral-like character, it presents a markedly extended surface area per unit of weight rendering it rapidly soluble in water of comfortable washing temperature. It further avoids a vitrified particle surface and contains no material of any appreciable quantity which is not immediately soluble in water under ordinary conditions. It also avoids the dustiness that in prior products proved annoying to users and is of advantageous moisture content. This product, referred to in the claims as a soap product, is furthermore predominantly a soap in contradistinction to washing powders or soap powders wherein the major portion of the solid ingredients is soda ash. Our product aforesaid contains principally soap with no more than a small portion of soda ash, in no case over 25%, and is produced by drying by evaporation and not by crystallization of sodium carbonate by cooling, as is the case with soap powders. The production of this product, moreover, obviates the necessity of high temperatures such as above referred to, and enables the attainment of far greater efficiency in the utilization of available heat with consequent small heat wastage.

The process for the production of the aggregated-particle coral-like soap powder of our invention comprises the spraying of a soap-paste into a current of a gaseous drying medium, such as air, which, while effectively and expeditiously drying the composition to the desired extent, does not involve a steam-generating inflating action. The comparatively low temperatures employed contribute to ease of control of the process, materially reduce fire hazards, and enable substantial economy in cost of apparatus and drying to be attained. In addition, these temperatures substantially avoid dehydration of the silicate in the soap composition to the point where such silicate becomes insoluble. They, moreover, permit the use of steam economically for heating the drying air, avoiding the use of combustion gases, or of oil fired heaters from which combustion gases may leak into the air, which gases, due to their carbon dioxide content, are likely to convert the sodium silicate in the product into insoluble silica.

Other features and advantages of our invention will be hereinafter described and claimed.

In the accompanying drawings:

Fig. 1 is a diagrammatic view illustrative of apparatus which may be employed for carrying out the process of the invention.

Fig. 2 is a longitudinal sectional view showing a form of spray nozzle which may be employed.

Figs. 3 and 4 are photo-microscopic views of the product.

Fig. 5 is a view showing a modified form of apparatus which may be employed in carrying out the process.

In carrying out the invention a soap paste is prepared and passed through spray nozzles at the top of a drying tower. The paste may be formed from pure kettle soap or from such soap mixed with other ingredients in a mixer 1 of conventional type. Mixtures varying in content from 100% pure commercial kettle soap to a content of 60% pure commercial kettle soap and 40% other ingredients have been successfully handled. The mixture may be diluted with water to any desired consistency. It may be conveyed from the mixer 1 by a pump 2 to a reservoir tank 3, from which it is transmitted by a pump 4 through steam heaters 5 to the atomizing nozzles 6 in the top portion of the tower 7. Usually the paste as sprayed contains from 40% to 50% water and is heated to approximately 200° F., although these figures may be varied.

The amount of soap mixture pumped to the nozzles may be conveniently regulated by operation of valve 8 controlling by-pass 9, whereby part of the material may be returned to the tank 3 depending upon the position of said valve.

In the nozzles the paste is subjected not only to the pressure of the pump 4, but also to the pressure of atomizing compressed air supplied to the nozzles from any suitable source. Pump pressures of from 60 to 75 lbs. per square inch and compressed air pressures of from 90 to 125 lbs. per square inch have been found satisfactory. The pressure of the compressed air supplied to the nozzles may be readily controlled by manipulation of a valve 6" in the compressed air line 6'. A suitable type of nozzle which may be employed is shown in Fig. 2, said nozzle comprising an opening 10 for the admission of the atomizing air, and an opening 11 for receiving the soap paste. The air passes through the interior of a hollow tubular member 12 containing a stationary helical element 13, while the soap paste, after entering a chamber 14, passes between stationary helical blades 15. The air and soap mixture thoroughly intermingle in the space 16 and leave the nozzle through restricted opening 17. Due to the action of the air the soap paste or mixture is atomized in very small particles. These particles impinge upon each other upon leaving the nozzle; said particles being sufficiently plastic to cohere and form agglomerates of highly irregular shape. These agglomerations, as will later be noted more particularly, consist of minute individual particles aggregated together with interstices therebetween and resembling coral in formation.

As the particles emerge from the nozzles they meet an ascending column of warm drying air supplied to the bottom portion of the tower 7 by a blower fan 18 through steam heaters 19. The rising column of air slows the speed of fall of the particles and maintains them in air suspension for an appreciable period. Through the steam coils 19 the temperature of the air, and hence its drying capacity, may be increased to such point

as will enable drying to be carried out at the desired rate; the temperature to which the air is heated depending upon how much material it is desired to dry for any given volume of air and how much moisture it is desired to remove. The 5 temperature of the air can be readily regulated to the desired point by controlling the amount of steam passing through the heaters 19 by any suitable valve, as will be apparent.

It will thus be noted that the amount of moisture dried from the material, or, conversely, the amount of moisture left in it, can be regulated at will without any change in the characteristic form of the product. A too high moisture content in the dried material leaves a product of a 15 sticky plastic nature, of no practical value commercially; while the material tends to become friable in character and prone to break down into dust when the moisture content is too low. A moisture content between 15% and 25% by weight 20 is desirable, the most preferable being around 18% to 22%, and this is readily obtainable. Through variation, individually or collectively, of the amount of drying air supplied per unit time, the temperature of the air, and the quantity of soap 25 paste supplied to the spray nozzles per unit time, the moisture content of the product may be brought to any desired value.

As the air passes upwardly through the tower in a direction opposite to that of the falling soap 30 particles, it is of course dropping in temperature due to its absorption of moisture from the soap particles and is becoming more saturated with moisture throughout its upward course. However, as its temperature drops and its moisture 35 content increases it is continually contacting with soap particles of higher moisture content so that its heat and drying capacity can be used to a maximum degree. The air exhausted from the equipment frequently has a relative humidity as 40 high as 75% which indicates the degree of efficiency in the use of heat and drying capacity of the air, and thus the efficient operation of the process from the standpoint of heat expenditure.

It will further be observed that the rate of production may be expeditiously controlled by simply varying the amount of paste pumped through the spray nozzles per unit time and correspondingly regulating the drying capacity of the air, as by appropriately changing its temperature. With 45 air supplied at the rate of 20,000 cubic feet per minute and a final moisture content in the product of 18% to 20%, an air temperature of 160° F. in front of the heaters 19 has been found suitable for a production rate of 1800 pounds per 50 hour (referring particularly to a product having the composition hereinafter specified by way of example), while an increase of said air temperature to about 200° F. enables the rate of production of said product to be approximately doubled. 55 The production rates obtained with these temperatures will, of course, vary with the moisture content of the atmospheric air.

Figures 3 and 4 illustrate microscopically the physical structure of the product, these views 65 showing typical agglomerate particles made up of smaller particles aggregated together with interstices therebetween. The sponge or coral like character of the agglomerates is clearly apparent and is wholly unlike the globular bead-like void-containing particles of the prior practice. Furthermore the individual particles which make up the agglomerates have no interior voids as do the globular bead or shell-like prior art particles. While certain portions in these views appear 70

somewhat rounded, this appearance is due to the fact that these portions were out of focus. They are actually of the same character as the remaining portions.

6 The agglomerated character of the particles contributes materially to low bulking weight or apparent specific gravity. In other words, due to the numerous interstices between the individual particles, the space per unit weight of the 10 agglomerate particle is large. The bulking weight is further lowered by the fact that the agglomerate particles are irregular with resultant spaces between the agglomerates in the package. One 15 advantageous soap product, of a composition later to be discussed more specifically and produced in accordance with this invention has been found to have an apparent specific gravity of between about .30 and .35 as packaged. In other words its bulking weight is between approximately 18 $\frac{1}{4}$  20 and 21 $\frac{1}{4}$  pounds per cubic foot.

The size of the agglomerates is illustrated by the following representative mesh analysis (made with standard screens):

|                           | Percent |
|---------------------------|---------|
| 25 Through 10 mesh screen | 100.00  |
| Through 20 mesh screen    | 85.00   |
| Through 40 mesh screen    | 53.00   |
| Through 60 mesh screen    | 33.00   |
| Through 80 mesh screen    | 10.00   |

30 The above percentages are by weight.

The drying air leaves the tower at the top through a duct 22, thence passing through a dust collector 23 containing screens 24 of canvas or other suitable material for removing any fine particles that may have been carried along with the air. The latter is discharged to the atmosphere by exhauster fan 25. The particles removed from the air by the screens 24 are collected in hoppers 26 from which they may be removed when desired. In this connection the screens aforesaid may be tapped or shaken automatically at regular intervals by any suitable and well-known apparatus. The particles removed from the hoppers 26 may be incorporated with the soap and other ingredients supplied to the mixer 1 and returned therewith through the spray nozzles 6.

The particles which descend through the drying air in the tower 1 are received upon conveyor belts 27, 28, whence they are passed through a chute 29 onto a conveyor belt 30. While on the latter said particles may be passed through a cooling chamber 30' wherein they are subjected to a current of air of suitable cooling temperature supplied by a fan or other source, for reducing their temperature to any desired extent. From conveyor 30 the particles are passed through a sifter 31 of appropriate mesh, for removing any oversized agglomerates, and are thence carried by conveyor 32 to conventional packaging machines.

The drying rate may be substantially expedited, and accurate control facilitated, by providing within the tower 1 an inner wall 33, having its intermediate section constricted, as shown, with respect to its end portions 34, 35. A passage of Venturi character is thus provided with consequent increase in velocity of the air through the major portion of its travel through the tower. If desired, the space 36 between the inner and outer walls of the tower may be supplied with warm air from fan 37 and heaters 38, as indicated, to prevent loss of heat by radiation from 75 the air within the inner wall 33 or to further

increase the drying capacity of said air by radiating heat thereinto through said inner wall. The outer wall 1 may be of suitable heat insulating construction.

By way of a specific example of the carrying 5 out of the invention there may be mixed together in the mixer 1 ingredients in substantially the following proportions:

|                                                                                                | Pounds | 10 |
|------------------------------------------------------------------------------------------------|--------|----|
| Kettle soap                                                                                    | 720    |    |
| Sodium silicate                                                                                | 144    |    |
| Sal soda                                                                                       | 117    |    |
| Scrap (which may be taken from hoppers 26 or from the material rejected by sifter 31, or both) | 100    | 15 |

To the above, water in an amount up to approximately 175 pounds is added to facilitate mixing. These materials are introduced into the crutcher or mixer 1 at a temperature such that 20 the temperature of the resultant paste is about 170°-175° F. As has been noted, the paste is pumped into reservoir 3; from which it is conveyed by pump 4 through heaters 5 into the spray nozzles 6. While the temperature of the paste 25 is raised to about 200° F. in the heaters 5, it may be pointed out that the heaters, though convenient, are not essential, and that paste at a temperature of 170° to 175° F. can be sprayed satisfactorily.

The paste prepared from the ingredients in the proportions above specified has approximately 30 the following formula:

|              | Per cent | 35 |
|--------------|----------|----|
| Water        | 46       |    |
| Dry soap     | 46       |    |
| Dry silicate | 5        |    |
| Dry soda ash | 3        |    |
|              | 100      | 40 |

After being sprayed and passed through the sifter 31 (the screen of which is of preferably 10 mesh, i. e., 10 openings per lineal inch, or 100 openings per square inch), the product is passed on to the packaging machines. The composition of the 45 finished product prepared from the ingredients in the proportions above specified by way of example, is approximately as follows:

|              | Per cent | 50 |
|--------------|----------|----|
| Water        | 20       |    |
| Dry soap     | 68       |    |
| Dry silicate | 7.5      |    |
| Dry soda ash | 4.5      |    |
|              | 100.0    | 55 |

The above percentages, as are all other percentages herein given, are by weight.

When the said product is taken from the cooling belt 30 it is generally at a temperature of about 80°-85° F. Said product has a bulking weight of between approximately 18 $\frac{1}{4}$  and 21 $\frac{1}{4}$  60 pounds per cubic foot, or an apparent specific gravity, when packaged, between about .30 and .35. The size of its agglomerates is illustrated by 65 the mesh analysis hereinbefore given.

The rapidity and completeness of solution of the aforesaid product is evidenced by the following test:

4 grams of said product was placed in 250 cubic centimeters of distilled water at a temperature of 70 100° F. and agitated for two minutes with an agitator operating at 200 revolutions per minute (the particular agitator employed being known 75

as the Cenco universal friction drive motor stirrer manufactured by Central Scientific Company, Chicago, Ill., and shown in their Bulletin No. 85, September, 1924). At the end of two minutes a portion of the solution was filtered through a cotton plug to remove undissolved soap particles, and 25 cubic centimeters pipetted from the filtered solution. The 25 cubic centimeters of filtrate were evaporated to dryness at 110° C. and the total soap therein determined. The weight of the portion remaining was then converted to percent dissolved product on the basis of the original sample, making proper adjustment for the original moisture content of the sample. From this test it was established that 98% of the product was dissolved in said two minute period. The aforesaid product (i. e., as withdrawn from the tower) is found to contain less than 0.10% matter insoluble in distilled water at 200° F., the average water insoluble matter amounting to only 0.04% or 0.05%.

It will, of course, be understood that the foregoing specific ingredients and proportions thereof are set forth only by way of example, and as hereinbefore indicated, the proportions may be widely varied, mixtures ranging from a content of 100% kettle soap to 60% kettle soap and 40% alkaline salts and other ingredients having been successfully spray dried in accordance with this invention and producing agglomerate particles having the characteristics above specifically discussed.

The bulking weight of the product will vary with the composition of the soap paste employed. For example, the bulking weight of the agglomerate particles produced by spraying a composition consisting of 100% pure kettle soap in accordance with the above described process, may be as low as 10 lbs.-12 lbs. per cubic foot. On the other hand, a decrease in the percentage of kettle soap and a corresponding increase of alkaline salts as compared with the example hereinbefore specifically given, will result in increase of bulking weight of the agglomerate particles. All specific gravities and bulking weights herein mentioned refer to the product as packaged.

As has been noted, during the ascent of the air through the tower it is absorbing moisture from the descending soap particles. Concurrently its temperature is dropping during its ascent. Thus, the air in the region of the nozzles is comparatively cool and moist and it is into this zone of increased moisture and diminished temperature that the atomization takes place from the nozzles. As a result the drying of the particles at this stage occurs at a moderate speed, leaving the particles of such plasticity that the particles will adhere upon impingement, but they are not sufficiently fluid to lose their identity through coalescence into a larger solid particle. This is in marked contrast to prior methods wherein the particles are sprayed into a zone of dry air of maximum temperature with consequent extremely rapid drying and immediate loss of plasticity preventing agglomeration. In addition, it is to be observed that due to the upward flow, in the present process, of the air against the downwardly moving particles, agglomeration is further facilitated since the downward progress of the finer particles is substantially impeded or prevented, affording increased opportunity for contact between these and other particles. In short, by delaying the passage of particles through the tower, the upwardly moving air current expedites materially agglomeration between the various

particles. Also, in the present process the soap is atomized from the nozzles in the form of a fine mist, with the result that the agglomerates formed are of the mesh sizes above indicated in connection with the finished product, while still containing a very large number of individual particles as sprayed; as distinguished from prior processes wherein the particles as sprayed are in the form of drops of substantial size and unagglomerated in the finished product.

As shown in Figure 5, the inner or Venturi-shaped wall 33 may be omitted and the drying air caused to travel upwardly throughout the full cross-section of the tower. The outer wall 1 is of suitable heat insulating construction.

The terms and expressions which we have employed are used as terms of description and not of limitation, and we have no intention, in the use of such terms and expressions, of excluding any equivalents of the features shown and described or portions thereof, but recognize that various modifications are possible within the scope of the invention claimed.

We claim:

1. A spray dried soap product comprising aggregates consisting of minute sprayed particles cohering together with interstices therebetween and without external void-defining shells, said aggregates being formed by the accretion of said minute particles and the cohesion thereof upon impingement while in suspension in a gaseous medium, said aggregates being subsequently dried while in suspension in a gaseous medium to reduce the plasticity thereof and prevent the adhesion of said aggregates to each other upon emergence from said medium, certain of said aggregates being of such size as to pass through a 60 mesh sieve and others comprising accretions of particles sufficient in quantity to prevent passage through a 60 mesh sieve but capable of passing through a sieve of 40 mesh.

2. A spray dried soap product comprising aggregates consisting of minute sprayed particles cohering together with interstices therebetween and without external void-defining shells, said aggregates being formed by the accretion of said minute particles and the cohesion thereof upon impingement while in suspension in a gaseous medium, said aggregates being subsequently dried while in suspension in a gaseous medium to reduce the plasticity thereof and prevent the adhesion of said aggregates to each other upon emergence from said medium, certain of said aggregates being of such size as to pass through a 60 mesh sieve and others comprising accretions of particles sufficient in quantity to prevent passage through a 60 mesh sieve but capable of passing through a sieve of 40 mesh.

3. A spray dried soap product comprising aggregates consisting of minute sprayed particles cohering together with interstices therebetween and without external void-defining shells, said aggregates being formed by the accretion of said minute particles and the cohesion thereof upon impingement while in suspension in a gaseous medium, said aggregates being subsequently dried while in suspension in a gaseous medium to reduce the plasticity thereof and prevent the adhesion of said aggregates to each other upon emergence from said medium, said product containing, by weight, over 15% water, and over 45% dry soap.

4. A spray dried soap product comprising aggregates consisting of minute sprayed particles cohering together with interstices therebetween and without external void-defining shells, said



here upon impingement, said aggregates being subsequently dried by evaporation during passage through said medium to reduce the plasticity thereof and prevent the adhesion of said aggregates to each other upon emergence from said medium.

15. A spray-dried soap product comprising aggregates consisting of minute sprayed particles cohering together with interstices therebetween and without external void-defining shells, said aggregates being formed by the accretion of said

minute particles and the cohesion thereof upon impingement while in suspension in a gaseous medium, said aggregates being subsequently dried while in suspension in a gaseous medium to reduce the plasticity thereof and prevent the adhesion of said aggregates to each other upon emergence from said medium, said product containing, by weight, over 15% water, over 45% dry soap, and less than 25% dry soda ash.

WILLIAM H. BURKHART. 10  
EUGENE T. MARCEAU.